

J. H. COTTON.

Manufacture of Iron Tubing.

No. 36,140.

Patented Aug. 12, 1862.

*Fig. 4.*



*Section of Tie*

*Fig. 3.*



*Fig. 2.*



*Section of Mandril with piece of Tube.*

*Fig. 1.*



*Section of Mandril.*

*Witnesses:*

E. B. Buckingham  
A. H. Cotton

*Invention:*  
J. H. Cotton

# UNITED STATES PATENT OFFICE.

JOSEPH H. COTTON, OF BOSTON, MASSACHUSETTS.

## IMPROVEMENT IN THE MANUFACTURE OF IRON TUBING.

Specification forming part of Letters Patent No. 36,140, dated August 12, 1862.

*To all whom it may concern:*

Be it known that I, JOSEPH H. COTTON, of Boston, Massachusetts, have invented certain new and useful Improvements in the Manufacture of Iron Tubing; and I do hereby declare that the following is a full, clear, and exact description of the same, reference being had to the annexed drawings, making a part of this specification, in which—

Figure No. 1 is a section of mandrel. Fig. No. 2 is a section of mandrel with piece of tube ready to be drawn. Fig. No. 3 is a front view of die. Fig. No. 4 is a section of die.

My improvement is applied in the following manner: I take short and thick iron tubes made in any of the usual modes for boiler-tubes. After annealing them they are dipped into dilute acid and then scoured, then into a bath of melted tin and tinned thoroughly both inside and outside. They are then drawn cold through dies upon steel mandrels, increasing them much in length, while decreasing them

in thickness, until the desired length and thickness are attained.

Tubes drawn in this manner are much superior to those made in any of the usual modes, being perfectly cylindrical and smooth upon both their inner and outer surfaces. The fiber, ductility, and malleability of the iron are much improved, in the same manner as rolled iron is improved in these respects by the cold-wire-drawing process.

Having thus fully described my invention, what I claim as new, and desire to secure by Letters Patent, is—

Coating iron tubes as set forth and subsequently drawing them while cold through dies, in the manner specified, thus producing a tube perfectly cylindrical and smooth upon both its inner and outer surfaces.

JOS. H. COTTON.

Witnesses:

E. B. BUCKINGHAM,  
FRANK B. COTTON.